

# UNITED STATES PATENT OFFICE.

WINFIELD S. POTTER, OF NEW YORK, N. Y.

## PRODUCTION, TREATING, AND ROLLING OF INGOTS OF MANGANESE STEEL.

975,371.

Specification of Letters Patent.

Patented Nov. 8, 1910.

No Drawing.

Application filed October 7, 1910. Serial No. 585,796.

*To all whom it may concern:*

Be it known that I, WINFIELD S. POTTER, a citizen of the United States, residing in the borough of Manhattan, city, county, and State of New York, have invented certain new and useful Improvements in Production, Treating, and Rolling of Ingots of Manganese Steel; and I do hereby declare the following to be a full, clear, and exact description of the invention, such as will enable others skilled in the art to which it appertains to make and use the same.

My invention relates to methods of producing, heating and rolling ingots of manganese steel, that is to say, steel usually containing from 10% to 15% or more of manganese, and from .80% to 1.25% or more of carbon. Steels for treatment in accordance with my invention may also have lower percentages of manganese, in which event the percentage of carbon may be diminished to advantage as the percentage of manganese is decreased. So also, for certain purposes, the steel may be provided additionally with a suitable proportion of some other metal or alloy, as for instance, chromium.

In the practice of my invention it is desirable to vary the details of the operation to some extent, as hereinafter indicated, to accord with the composition of the metal and the character and dimensions of the article to be produced or the shape to be rolled. In all cases, however, I have found that there are certain underlying principles and laws which must be duly taken into consideration in the treatment of the metal in accordance with the invention if the best products and the greatest degree of economy are to be secured. These principles and laws and their utilization in the practice of the invention I will now proceed to set forth, at first dealing with the steel, for the sake of simplicity, as a ternary compound of iron, manganese and carbon; although the steel will usually contain small quantities of such elements as phosphorus, sulfur and silicon and may also, as above indicated, contain other metals in addition to the iron and manganese.

When the liquid metal is cast and is permitted to freeze, certain substances or mixtures separate out of the mass and freeze first, with the formation of crystals of a composition nearly or quite the same as the average analysis of the metal poured, depending principally upon the composition

of the steel which has been made. These first formed crystals are composed of iron with manganese alloyed with or in solution in the iron and will be hereinafter termed mix crystals. The mix crystals forming in a steel containing carbon have in solution a proportion of carbids of iron and manganese.

When the carbon content of the metal is considerable, a secondary structure is produced at a lower temperature than the freezing point of the mix crystals, by a separation, from the balance of the metal, of alloys richer in manganese and carbon than the average of the whole mass. This richer metal crystallizes in the open spaces of the network of mix crystals previously formed. The portions last freezing, (the eutectic), consist of one or more carbids of iron and manganese, and for convenience will be hereinafter referred to as carbids. The carbids themselves may also be separated by selective freezing, so that certain microscopic layers may be formed containing manganese approximately 40% and carbon 6% or more, while other layers may form containing manganese about 20% and carbon 4% or more, in a mass of which the average analysis is for example manganese 13% and carbon 1.40%. The carbids containing the higher manganese percentage freeze first, that is, at the higher temperature. These separations are most pronounced in steel of high manganese content which has frozen slowly and when the steel is hyper-eutectoid, that is, when it contains carbon in excess of the eutectoid ratio for the percentage of manganese present. The eutectoid ratio will for the purposes of this specification, be defined as that percentage of carbon for a given manganese percentage which produces a quantity of carbids equal to the amount which the mix crystals are capable of taking into solid solution when the mass is heated to a temperature above the melting point of the eutectic, but below the melting temperature of the mass. Steel containing more carbon than this ratio will be classed as hyper-eutectoid, and steels containing less as hypo-eutectoid.

The proportion of carbids in the whole mass when it is frozen depends upon the total average percentage of manganese in the metal before freezing, and more particularly upon the total average percentage of carbon. Thus, steel containing 12% of man-

ganese with a proportion of carbon as high as .85%, or a higher proportion of carbon, will, when frozen in a given manner and at a certain rate, have less free carbids than steel containing the same percentage or content of carbon and containing but 10%, for example, of manganese. The amount of the carbids selectively frozen out in the whole mass is also a function of the rate of freezing, 10 and the distribution of the carbids throughout the mass is likewise dependent principally thereon, the rate of freezing being determined by additional considerations such as the temperature at which the metal is poured, the chilling capacity of the walls of the mold, the dimensions of the ingot to be cast, and the like.

The outer layer of the ingot is usually fine in grain and consists of small mix crystals 20 surrounded by very thin layers, if any, of carbids. Within this fine-grained skin, a structure, normal to the surface of freezing, forms, in which the mix crystals are built one upon the other in nearly straight lines, 25 and the resulting columns or dendrites are separated by layers of crystals of the carbids. The remaining interior portion of the mass is made up of a very uniform network of the mix crystals filled in with the 30 carbids.

When the period of freezing is long, the layers of carbids forming between the dendrites are heavy, and this dendritic portion of the mass may even be hyper-eutectoid. 35 when the remaining portions of the ingot are hypo-eutectoid. Very high carbon steel cooled slowly in the mold will produce ingots highest in manganese in the dendritic portion, and highest in carbon in the central 40 portion, while hypo-eutectoid steel cooled slowly in the mold results in ingots having both manganese and carbon highest in the zone of dendrites.

When the ingot is frozen throughout rapidly, the local carbid enrichments are less and are more nearly equal between the different parts of the ingot, than when the period of freezing is long; so that the average metal in the dendrite portion of the ingot may show, by 50 analysis, the same manganese and carbon as the central portion, and both may contain the same percentage of these elements as the skin or first layer frozen. This equality in average composition between the different 55 localities in the mass cannot be secured in a large ingot when the carbon of the steel is at or above the eutectoid ratio. On this account, when manganese steel of a specified carbon content is desired, the manganese per 60 cent. should be raised to equal or exceed the eutectoid ratio, and the steel should be cast in the smallest or thinnest ingot sections which will produce the required shape with the proper amount of mechanical work, that 65 is, the amount of mechanical work which

will weld and unite the particles and properly break down any coarse structures or crystals which may be present.

When the steel is heated to temperatures above the change point lying usually in the neighborhood of  $1025^{\circ}$  C. the carbids become weak in consequence of the close approach to their several melting temperatures and at about the same temperature, that is, at about  $1025^{\circ}$  C., the carbon of the carbids begins to distribute into the mix crystals. As the temperature is raised above the change point the outlines of the carbid areas are gradually lost and the carbids finally disappear altogether by absorption into the balance of the mass if the heating is sufficiently prolonged, and providing the specimen is not hyper-eutectoid. The freezing grains are also broken up during the absorption of the carbids in such a manner that the mass is stronger, the contact of the mix crystals being no longer broken by the weak cleavage planes of the carbids.

If the mix crystals in any part of the ingot form such a proportion to the local carbids that the mix crystals can be made to take into solid solution the excess carbon of these local carbids, the metal which thereafter remains in the position of the original carbids will have a carbon content more nearly equal to the average of the whole mass, but will have a higher percentage of manganese. This carbid residual will be rendered ductile in consequence of its loss of excess carbon, although its ductility will be less at a given temperature than that of the adjoining mix crystals of lower manganese content; but if the time and temperature have been sufficient the carbid residuals will recrystallize homogeneously with the other mix crystals. The ductility of the whole mass will still depend upon the quantity and original character of the carbids and will be greater as manganese and carbon were originally lower in the poured metal and as the freezing was more rapid.

If the heating to temperatures above  $1025^{\circ}$  C. or thereabout, is sufficiently prolonged, the mix crystals will first absorb a portion or all of the excess carbon of the carbids and by still longer heating the excess manganese of the carbids will also to some extent be distributed. By prolonged heating, at temperatures below the melting point of the carbids, the whole mass may in this way be rendered sufficiently ductile for rolling at temperatures ranging from  $1025^{\circ}$  C. to  $1150^{\circ}$  C. If, however, the whole mass is raised to a temperature above the melting point of the carbids, or carbid residuals, as for example, a temperature of  $1175^{\circ}$  C., a portion or all of the carbids in any locality in the ingot will be taken into solid solution by the adjoining local mix crystals. If, in any locality, the steel is hyper-eutectoid the

excess carbids may, by long heating, be in part distributed throughout the mass and away from their original location, providing the poured steel has the eutectoid ratio 5 or a lesser amount of carbon. When the melted composition is, for example 12% manganese and 1.40% carbon, the excess carbids render the metal very weak at all temperatures above 1050° C. or thereabout. 10 It is, therefore, important that the steel should not be hyper-eutectoid, if the metal must be rolled into shapes requiring considerable ductility of the ingot, and requiring a high rolling temperature. In the case 15 of a typical steel containing about 12% of manganese, a percentage greater than about 1.25% of carbon would make the steel hyper-eutectoid. This eutectoid carbon percentage depends also on the content of sili- 20 con and of chromium and the like. When the percentage of carbon in a given locality is much greater than this amount, but when the total proportion is not hyper-eutectoid, the uniform distribution of carbon is to be 25 brought about only by a very long period of heating, which for most purposes is not commercial. Generally, the metal is satisfactory if it contains 1.15%, or even a less proportion of carbon, and when the per- 30 centages of carbon range from 1% to 1.15% and the freezing has been rapid, the re-distribution of carbon may usually be effected in from one to four hours heating at tem- 35 peratures ranging from 1175° C. to 1100° C. 40 The melting point of the carbids first frozen out ranges from about 1120° C. to 1250° C., rising with their manganese content; while, for a given manganese per cent., the carbon having already been in part dif- 45 fused into the balance of the mass during a reheating operation, the melting point of the remaining metal in the locus of the origi- 50 nal carbid will now be higher. This rise in melting point temperature by loss of car- 55 bon usually stops at about 1160° C., when the whole mass has been quickly frozen and when it is hypo-eutectoid steel. Steel which is above or near the eutectoid ratio and which has been slowly frozen, and particu- 60 larly such steel when it has afterward been slowly heated to even as high as 1200° C., may still contain unmelted carbid residuals which may require a temperature as high as 65 1250° C. for their melting, solution and dif- fusion.

To determine whether steel of a given composition is hyper-eutectoid or hypo-eutectoid within the significance of these terms as used in this specification, the following procedure will suffice: A casting of the steel in question is made, removed from the mold, and a test piece is broken off and examined. Another test piece is reheated to the proposed rolling temperature, held at this temperature for a time which would be

commercial in the heating of ingots or blooms, and is then rapidly cooled. The re-heated steel is now examined. Fractures are obtained which run in various directions, such that the freezing structures, if any still 70 remain, are exhibited. Sections of the metal are also examined under the microscope. If carbids or their residuals are still in evi- 75 dence, separating the freezing grains or structures or their original outlines, or if considerable carbid areas appear within the grains of the mix crystals, the steel is hyper-eutectoid for the temperature and time used. A further test at a higher temperature or a longer commercial period of heating still 80 failing to show that any suitable rolling temperature or suitable time in heating will effect the solution and disappearance of the carbids, it can be decided that the steel can only be rolled by first cooling the exterior 85 portions of an ingot or by using moderate drafts and avoiding considerable elonga- 90 tions of the ingot before its exterior portions are rendered ductile.

In order to illustrate the method to be 90 employed in practicing my invention, I will now describe a specific instance of the pro- 95 cedure. Thus, in order to reduce the cost of manufacture and produce the best prod- 100 uct when a rail containing 12% manganese is required, the steel, which should be as free as possible of dissolved oxids, is made to contain a percentage of carbon well be- 105 low the eutectoid, as, for instance, 1.15% or less of carbon, and is poured into molds 110 comprising chills of sufficient mass to cause the steel to set rapidly, the steel being 115 poured at a temperature preferably not more than 50° C. above its freezing or set- 120 ting point, *i. e.*, at a temperature of 1400° C. or less. The ingots are allowed to cool in 125 the molds until they have frozen to or nearly to their central portions. They are then still further permitted to cool, if necessary, until the freezing structures which may 130 still be present have so cooled and solidified, and until their interior portions have so cooled, that, when placed in the heating fur- 135 nace, the ingots will not be heated in their outer portions too rapidly by transmission to said outer portions of the interior heat. The dendrites of the ingots are, however, 140 preferably broken down and reconstructed, by permitting the dendritic zone to be slowly or evenly reheated to the necessary tempera- 145 ture for that purpose by heat from the in- 150 terior portions, before the removal of the ingots from the molds. The ingots are then placed in the soaking pit or heating furnace, with an average temperature of 1000° C. to 155 1100° C., and are heated, during a period of from half an hour to an hour, to an average 160 temperature lying between 1150° C. and 1200° C., until the carbids are distributed 165 into the mix crystals. This will usually be 170

accomplished in between one and two hours, depending upon the original composition, and the rate of freezing, the lesser time being required for the lower carbon and manganese contents and the most rapid freezing. The steel is now in a state of chemical equilibrium, and will have a uniform fine gamma-iron structure, and the ingots may be taken to the mill and rolled with heavy reduction in the first passes and with reductions thereafter as desired, without any other preliminary cooling of the exterior portions than that which is usually incident to the transfer. This usually results in dropping the exterior temperature about 20° to 50° C.

The rail, as it leaves the rolls, should be cooled rapidly to avoid separation of carbids in the steel, and to avoid the structural rearrangement caused by slow cooling to about 600° C., whether the rolling of the ingot to the finished shape has taken place in a single heat, or in two heats (by the preliminary production of a bloom). The cooling of the finished product should proceed at a moderately rapid rate to below 600° C., (preferably below 400° C.) as by means of a water shower on some portion of the mill table or hot bed. The cooling will usually be sufficiently rapid with such steel if it is done in five or six minutes or less in the mill, and one minute or less under the water shower, the essential feature being to get the ingot or bloom in a condition of chemical equilibrium and to then roll and cool either with mechanical work or with rapid cooling going on continuously until the rail has temperatures preferably below 400° C.

If it is found necessary to pour the steel at a higher temperature, or in the large ordinary iron molds and to get the ingots to the soaking pits with a dendritic structure still remaining in their exterior portions, the heating from 1025° C. upward, until the eutectic in the outer portions of the ingot has entered into solid solution, should be longer than as above stated to avoid any disintegration of the dendritic portions. For the reason that ingots poured at high temperatures have, as previously stated, considerable local enrichments in their exterior portions, it will usually be found safest to lower the temperature of the outer portions of the ingot to 1120° C. or a lower temperature depending upon the original composition, before the ingot enters the rolls. Also when a high maximum temperature has been maintained for a long time, the cooling step will sufficiently strengthen the mass by shrinking and welding the grains of steel.

Manganese steels containing considerably less carbon than the eutectoid ratio, and especially those steels which are without considerable free carbide areas when slowly

cooled, as, for example, a steel containing manganese 13%, carbon .30%, may be rolled satisfactorily at temperatures between 1100° C. and about 1225° C. by first evenly heating to reconstruct the outer portions of the ingot, and then somewhat cooling or first lightly rolling if the maximum temperature was above 1200° C. for example, and if a coarse loose grain is present. But such steels are too ductile when cold for most purposes for which manganese steel is employed. Indeed, for many uses, the steel should be made hyper-eutectoid.

When it is desirable to produce rolled shapes from hyper-eutectoid steel, the preliminary heating above 1025° C. and up to the maximum temperature employed should be very slow. The maximum temperature in the case, particularly of large ingots, which have cooled slowly, should be upward of 1200° C., and the outer portions of the ingot and to a considerable depth as, for example, two or more inches measured inward from the surface of the ingot, should be cooled to a temperature considerably lower than the freezing temperature of the remaining undissolved carbids. When the ingots of hyper-eutectoid steel are of a moderate thickness, the necessary ductility for a preliminary rolling may be obtained by heating to a temperature which will in part distribute the excess carbon of the high manganese carbids as, for example, a temperature of 1100° C. or slightly less, until the redistribution of carbon has gone as far as possible, which will usually require about four hours at the maximum temperature. The preliminary breaking down of the grain by a light blooming operation is then executed, and the slab or other bloomed shape is then reheated to a temperature usually ranging from 1100° C. to 1150° C. and depending upon the amount remaining of undissolved carbids, the highest permissible temperature being lower as the proportion of carbids not capable of re-solution is greater. Steel of this character should be finally quenched in water at a temperature preferably between 1025° C. and 1075° C. and, if necessary, should be reheated to within this range of temperature for quenching.

If the steel is found to be eutectoid or hypo-eutectoid, in making examination of a trial casting as previously described, it may be rolled by heating to the predetermined temperature and for the predetermined time, and without preliminary cooling or preliminary compression or otherwise welding the exterior portions of the ingot. If the steel consists of large loosely cohering grains of gamma-iron, but of different size and arrangement from the freezing structures found in the casting before reheating, the temperature, or the duration of the heating

at the maximum temperature has been excessive for rolling without first welding or cooling. If, by further testing at lower temperatures the reconstruction of the metal cannot be effected without obtaining evidences of overheating, then the steel of given composition can only be rolled by cooling its outer portions to below the freezing point of the undissolved eutectic, or by first lightly 10 rolling and compressing, or both. When steel of eutectoid or of softer composition is investigated, as above indicated, it is frequently converted into a fine uniform gamma-iron structure by a temperature and time 15 considerably less than that which produces the overheated condition. Ingots of such steel may be rolled to advantage with a higher temperature in their exterior than in their interior portions. Furthermore, I 20 have found that when steel containing about 12% of manganese and 1.10% of carbon is cast at temperatures ranging from 1350° C. to 1550° C., depending upon the size of the ingot, the interior portions of the ingot may 25 be suitably reconstructed by heating to temperatures above 1120° C., and the exterior portions may be reconstructed by heating to the same or a higher temperature, as for example 1175° C., the higher temperature for 30 the higher casting heat and the slower freezing. So that, when large ingots of eutectoid or softer steel have been cast at more than about 50° C. above the freezing point of the metal, the outer portions of the ingot usually 35 require a higher temperature for their reconstruction in a given time. As the evidences of overheating seldom appear until the steel is heated to about 1200° C. it is 40 usually a safe procedure to heat the outer portions of the ingot to any temperature below this point, or even to heat the outer portions for a short time to temperatures somewhat above 1200° C., while holding the interior temperature somewhat lower so as to 45 maintain a strong supporting central core; as, for example, heating the ingot to 1190° C. at its surface, and 1140° C. at its center, or, for example, heating the ingot until the interior portions are strong and ductile with 50 a temperature of 1150° C. and bringing the outer portions to 1200° C. for a few minutes, and then taking the ingot from the heating furnace to the rolls. This method has the further advantage of avoiding an excessive 55 central temperature, caused by the combined effects of the initial heating at the center and the heat of internal friction generated during rapid rolling.

Having thus described my invention, what 60 I claim is:

1. The method of preliminarily treating and subsequently rolling manganese steel ingots containing carbids, consisting in heating the ingot to temperatures above the 65 change point at which the carbon begins to

be rapidly absorbed from the carbids by the mix crystals and until the mix crystals have absorbed substantially the maximum amount of carbon that they are capable of abstracting at the temperature employed, 70 and continuing the heating until the carbid residuals are recrystallized, forming with the mix crystals a gamma-iron structure, and then rolling the ingot; substantially as described. 75

2. The method of preliminarily treating and subsequently rolling manganese steel ingots containing carbids, consisting in heating the ingot to temperatures above the change point at which the carbon begins to 80 be rapidly absorbed from the carbids by the mix crystals and until the mix crystals have absorbed substantially the maximum amount of carbon that they are capable of abstracting at the temperatures employed, 85 and continuing the heating until the carbid residuals together with any undecomposed carbids are recrystallized, forming with the mix crystals a gamma-iron structure, and then rolling the ingot; substantially as de- 90 scribed.

3. The method of preliminarily treating and subsequently rolling manganese steel ingots containing carbids, consisting in heating the ingot to temperatures above the 95 change point at which the carbon begins to be rapidly absorbed from the carbids by the mix crystals and until the mix crystals have absorbed substantially the maximum amount of carbon that they are capable of 100 abstracting at the temperatures employed, continuing the heating until the carbid residuals are recrystallized, forming with the mix crystals a gamma-iron structure, welding the gamma-iron crystals into a more cohesive ductile mass before subjecting the ingot to heavy reductions, and then rolling the ingot; substantially as described. 105

4. The method of casting, treating, and subsequently rolling manganese steel ingots 110 containing carbids, consisting in pouring the metal at a temperature not more than 50° C. above its freezing point, freezing the metal at such a rate as to avoid considerable variations in composition between different localities of the ingot and so as to avoid considerable separation of carbids, heating the ingot to temperatures above the change point at which the carbon begins to 115 be rapidly absorbed from the carbids by the mix crystals and until the mix crystals have absorbed substantially the maximum amount of carbon that they are capable of abstracting at the temperatures employed, and continuing the heating until the carbid residuals are recrystallized, forming with the mix crystals a gamma-iron structure, and then rolling the ingot; substantially as de- 125 scribed.

5. The method of casting, treating, and 130

subsequently rolling manganese steel ingots containing carbids, consisting in pouring the ingot from metal substantially free of oxids, and at a temperature not more than 50° C. 5 above its freezing point, freezing the metal at such a rate as to avoid considerable variations in composition between different localities of the ingot and so as to avoid considerable separations of carbids, heating the 10 ingot to temperatures above the change point at which the carbon begins to be rapidly absorbed from the carbids by the mix crystals and until the mix crystals have absorbed substantially the maximum amount 15 of carbon that they are capable of abstracting at the temperatures employed, and continuing the heating until the carbide residuals are recrystallized, forming with the mix crystals a gamma-iron structure, and then 20 rolling the ingot; substantially as described. 6. The method of preliminarily treating and subsequently rolling manganese steel ingots containing carbids, consisting in heating the ingot to temperatures above the 25 change point at which the carbon begins to be rapidly absorbed from the carbids by the mix crystals and until the outer portions of the ingot have a uniform strong gamma-iron structure, and then rolling the ingot; sub- 30 stantially as described. 7. The method of preliminarily treating and subsequently rolling manganese steel ingots containing carbids, consisting in heating the ingot until the carbids have been 35 partly decomposed and heating further to temperatures above the melting point of the resulting carbide residuals until said residuals have been taken into solution by the mix crystals, and then rolling the ingot; substantially as described. 8. The method of preliminarily treating and subsequently rolling manganese steel ingots containing carbids, consisting in heating the ingot to temperatures lying between 40 1120° C. and 1200° C. until the excess carbon of the carbids is redistributed throughout the mass and until the carbide residuals have been taken into solid solution to sub- 45 stantially the limit of the capacity of the mix crystals for such solution at the temperature employed and thereby rendering the ingot ductile and coherent, and then rolling the ingot; substantially as described. 9. The method of preliminarily treating and subsequently rolling manganese steel ingots containing carbids, consisting in heating the ingot until the carbids have been 50 partly decomposed and heating further to temperatures above the melting point of a portion of the residuals resulting from decomposition of the carbids, causing the unmelted portion of the residuals to dissolve in the melted portions, and maintaining the temperature until the carbide residuals have 55 been distributed throughout the remainder

of the mass to substantially the limit of the capacity of such remainder for effecting such solution at the temperature employed, and then rolling the ingot; substantially as described.

10. The method of preliminarily treating and subsequently rolling manganese steel ingots containing carbids, consisting in heating the ingot to a predetermined temperature above 1120° C. and continuing the heating operation for a predetermined time such that any free carbids will be taken into solution in the mix crystals, and then rolling the ingot; substantially as described.

11. The method of preliminarily treating and subsequently rolling ingots of manganese steel of hypo-eutectoid composition, consisting in heating the ingot until the carbids have been partly decomposed and heating further to temperatures above the melting point of the resulting carbide residuals until said residuals have entered into solid solution in the mix crystals, and then rolling the ingot; substantially as described.

12. The method of preliminarily treating and subsequently rolling manganese steel ingots of hypo-eutectoid composition, consisting in heating the ingot until the carbids have been partly decomposed and heating further for a predetermined time within a predetermined range of temperature until the carbide residuals have been absorbed by the mix crystals, with the production of a uniform gamma-iron structure, and rolling the steel with the distribution of temperature then obtaining; substantially as described.

13. The method of preliminarily treating and subsequently rolling manganese steel ingots, consisting in heating the ingot to temperatures above the change point at which the carbon begins to be rapidly absorbed from the carbids by the mix crystals, heating the outer portions of the ingot to higher temperatures until said outer portions have a uniform strong gamma-iron structure, and then rolling the ingot; substantially as described.

14. The method of preliminarily treating and subsequently rolling manganese steel ingots containing carbids, consisting in heating the ingot to temperatures above 1120° C. until the ingot has a substantially uniform gamma-iron structure throughout, which temperatures if above 1200° C. in the outer portions shall be maintained for a short time only, and then rolling the ingot; substantially as described.

15. The method of preliminarily treating and subsequently rolling manganese steel ingots, consisting in heating the ingot to temperatures above 1120° C., thereby forming in the outer portions of the ingot a strong gamma-iron structure, heating the said outer portions to higher temperatures, which lat- 125 130

ter temperatures if above 1200° C. shall be maintained for a short time only, and then removing the ingot to the mill and rolling said ingot; substantially as described.

ture, then rolling, and cooling the resulting shape at a rate sufficiently rapid to avoid 35 structural rearrangement during the cooling; substantially as described.

16. The method of preliminarily treating and subsequently rolling hypo-eutectoid manganese steel ingots, consisting in heating the ingot of hypo-eutectoid steel to temperatures above those at which the carbids and 10 carbid residuals are distributed throughout the mass, and until said distribution has been effected, then rolling the ingot, and cooling the finished shape at a rate sufficiently rapid to avoid separation of carbids; 15 substantially as described.

17. The method of preliminarily treating and subsequently rolling hypo-eutectoid manganese steel ingots, consisting in heating the ingot to temperatures above those at 20 which the carbids and carbid residuals are distributed throughout the mass, and until said distribution has been effected, preserving said distribution until the rolling operation begins, then rolling and cooling the finished shape at a rate sufficiently rapid to 25 avoid structural rearrangement during the cooling; substantially as described.

18. The method of preliminarily treating and subsequently rolling manganese steel, 30 consisting in heating a mass of manganese steel having carbids in solution in the mix crystals to temperatures above 1120° C. until the mass has a uniform gamma-iron struc-

ture, then rolling, and cooling the resulting shape at a rate sufficiently rapid to avoid 35 structural rearrangement during the cooling; substantially as described.

19. The method of casting, treating and subsequently rolling manganese steel ingots, 40 which consists in pouring the ingot from metal substantially free from oxids, freezing the metal at a rate to avoid considerable variations in composition between different localities of the ingot and to avoid considerable separation of carbids, reconstructing the 45 outer portions of the ingot by raising their temperature slowly and evenly while still in the mold, then transferring the ingot to a soaking pit and heating until by redistribution of their carbon and carbid residuals the 50 outer portions of the ingot have dropped below the hyper-eutectoid ratio, heating until the mix crystals of the entire mass have absorbed substantially the maximum amount of carbon that they are capable of abstract- 55 ing at the temperature employed and until the carbid residuals throughout are recrys- tallized forming with the mix crystals a gamma-iron structure, and then rolling the ingot; substantially as described. 60

In testimony whereof I affix my signature, in presence of two witnesses.

WINFIELD S. POTTER.

Witnesses:

JOHN C. PENNIE,  
WILLIAM H. DAVIS.